

March 2, 1943.

A. R. DEVEREUX

2,312,324

OSMIUM COMPOSITION

Filed April 21, 1941

*Fig. 1.*



*Fig. 2.*



INVENTOR.

Andrew R. Devereux.  
BY Chilton, Wiles, Davies & Hirsch.  
*Atty's.*

## UNITED STATES PATENT OFFICE

2,312,324

## OSMIUM COMPOSITION

Andrew R. Devereux, Chicago, Ill., assignor to  
 Goldsmith Bros. Smelting & Refining Company,  
 a corporation of West Virginia

Application April 21, 1941, Serial No. 389,638

4 Claims. (Cl. 75—172)

This invention relates to a composition consisting predominantly of osmium, in which the osmium is in a felted acicular non-dendritic form.

The degree of smoothness to which a metal surface may be polished depends upon the microscopic texture of the metal itself. This is particularly true with respect to pen point alloys because of the duplex character of the micro-structure. All of the better grade pen point alloys contain at least two structural components of different hardness. When alloys of this type are polished, there results, in consequence of the preferential wearing of the softer aggregate, a relief effect in which the harder constituent appears in the form of ridges. By means of the present invention a structure is developed in which the particles of the harder phase are so closely interwoven or interlaced with the softer phase, that perceptible isolated regions of the soft constituent are no longer perceptible.

In Devereux and Pfanstiehl Patent No. 2,206,616 is described an osmium composition consisting predominantly of osmium, in which the osmium is in the form of discrete particles, non-dendritic in arrangement and form. The product there described was produced by the heat treatment of pressed powder particles of osmium and other metals. The present invention relates to an improvement thereon and more particularly to a product produced by heat treating a composition in such manner as to render the osmium particles acicular in form and felted in arrangement.

By following the present process there is a tendency for the matrix to dissolve a portion of the osmium, and for the osmium particles to dissolve a portion of the matrix, undergoing in the process a very considerable change in form and arrangement, without, however, becoming dendritic. During the change, the matrix, being smaller in quantity than the osmium, has a tendency to disappear, and the final product is substantially free from isolated areas of the relatively soft matrix material. On the other hand, the particles of the osmium-rich phase become rod-like or acicular in form, and interlaced or felted in arrangement.

The preferred alloy consists of approximately 85% osmium and 15% platinum. The product is prepared by intermixing osmium and platinum powders in the correct proportion, pressing them together under heavy pressure, and then sintering the resulting crude mass at a suitable temperature in an inert atmosphere.

The transformation of the material is carried

on above 2900° F. and is completed by maintaining the product at approximately 3100° F. for 2 hours.

The structure of the resulting composition is illustrated in the drawings, in which Figure 1 is a photolithograph of an area of the composition which has been magnified about 2,000 diameters; and Figure 2 is a corresponding photolithograph which has been magnified about 500 diameters. 10 It will be observed in both photographs that the osmium particles are in the form of rods 10 which are felted or interlaced. It will be noted that even at a magnification as high as 2,000 diameters there are no discrete regions of soft constituent perceptible.

The present invention is not limited to the particular matrix here described, nor to the particular proportions of osmium-rich phase and matrix set forth in the specific example, so long as the osmium is predominant in proportion and the structure produced is that herein set forth. 20 This is likewise true of the physical conditions attending the processing, such as the pressure of compacting, the temperature of sintering, etc.

For example the replacement of some of the platinum by small proportions of rhodium has a tendency somewhat to coarsen the structure, although the general crystal shape is preserved. The addition of tungsten on the other hand has a tendency to refine the structure by making the crystal sizes considerably smaller, although the general shape thereof is preserved.

The use of the narrow heat treating range here specified, in combination with the compositions 35 here given, likewise has a tendency to reduce porosity, the materials prepared in accordance with the present invention being essentially non-porous.

As stated, the material herein described is of particular value for use in pen points, in connection with which the interlaced acicular masses of osmium-rich phase, held in the almost imperceptible body of matrix, produce long wear and a highly satisfactory writing surface.

The foregoing detailed description has been given for clearness of understanding only, and no unnecessary limitations should be understood therefrom.

What I claim as new, and desire to secure by Letters Patent, is:

1. An osmium alloy consisting predominantly of an osmium-rich phase in the form of acicular crystals in interlaced arrangement held together by a matrix consisting essentially of platinum

metal, the matrix being characterized by the absence of isolated masses of matrix.

2. A non-porous osmium alloy consisting entirely of platinum group metal except for impurities which do not affect the characteristics of the alloy, containing more than 50% and not substantially more than 85% of osmium, and the balance being substantially all platinum metal, there being an osmium-rich phase in the alloy in the form of interlaced acicular crystals non-dendritic in arrangement, and an osmium-lean phase of platinum matrix metal characterized by the absence of isolated masses of matrix, the matrix phase holding together the osmium-rich phase.

3. An alloy as set forth in claim 2, in which the osmium content is 85% and the platinum is 15%.

4. An osmium alloy consisting entirely of platinum group metal except for impurities which do not affect the characteristics of the alloy, containing substantially 85% of osmium and the balance being substantially platinum metal, there being an osmium-rich phase in the alloy in the form of interlaced acicular crystals and an osmium-lean phase of platinum matrix metal characterized by absence of isolated masses of matrix, the matrix phase holding together the osmium-rich phase.

15

ANDREW R. DEVEREUX.